

## UNITED STATES PATENT OFFICE.

IRVIN W. HUMPHREY, OF KENVIL, NEW JERSEY, ASSIGNOR TO HERCULES POWDER COMPANY, OF WILMINGTON, DELAWARE, A CORPORATION OF DELAWARE.

## PINE-OIL PRODUCT AND PROCESS OF MAKING SAME.

No Drawing.

Application filed August 17, 1925. Serial No. 50,839.

The object of my invention is to provide a nitrocellulose lacquer or varnish. Another object of my invention is to provide a nitrocellulose lacquer containing an ingredient

5 which will serve to some extent as a substitute for castor oil and other substances which are used to produce films of high flexibility. Another object of the invention is to produce a nitrocellulose lacquer ingredient 10 which may be used as a substitute, in whole or in part, for amyl or butyl acetates and which can be produced more cheaply, thereby effecting a saving in the cost of manufacturing the lacquer.

15 Pine oil is known to be a complex mixture of different substances, including terpineol, methyl chavicol, borneol, fenchyl alcohol, terpene hydrocarbons and smaller amounts of several other bodies. Pine oil

20 itself has no colloidizing action upon nitrocotton, and its individual constituents also possess little colloidizing power. However, certain of these constituents, notably borneol and fenchyl alcohol, yield, on oxidation, the 25 ketones camphor and fenchone respectively, the former being a well known colloidizing agent for nitrocellulose.

30 Pine oil contains above five per cent of borneol, and approximately as much fenchyl alcohol. These two alcohols cannot be easily isolated from pine oil in a high degree of purity by means of fractionation because of the nearness of their boiling points with those of some of the other constituents of 35 pine oil.

As set forth in an application filed by me November 22, 1924, Serial No. 751,682, I have found that it is feasible to treat pine oil with certain oxidizing agents and obtain 40 a liquid, which may be designated oxidized pine oil, which exhibits considerable colloidizing action on nitrocellulose. When pine oil is oxidized under proper conditions, it may contain approximately ten per cent of the 45 ketones camphor and fenchone and, in addition, small amounts of other oxidized substances which colloid nitrocellulose. Another portion of the pine oil is oxidized to inert bodies, but the operation may be so conducted that a great portion of the pine oil

remains unaltered, serving as a diluent to the active colloidizing agents but possessing a strong solvent power for resins.

A solution of nitrocellulose may be prepared in straight oxidized pine oil, but on account of the rather high boiling range of 55 oxidized pine oil, which is comparable to that of pine oil itself, it is usually desirable to add large proportions of lower boiling liquids. The latter may be either solvents 60 or non-solvents for nitrocellulose. Examples of solvents are acetone and butyl acetate, and of non-solvents, alcohol and benzene. It is possible to incorporate a large proportion 65 of a non-solvent in the vehicle without precipitating the nitrocellulose. Alcohol, even if it contains as much as five per cent of water, is found to be a desirable diluent from the standpoint of increasing the colloidizing action of oxidized pine oil. Even 70 if as much as several volumes of alcohol are added, the colloidizing action of oxidized pine oil is accelerated to a remarkable degree.

Several oxidizing agents have been employed in preparing oxidized pine oil. 75 Nitric acid is well adapted for use on a fraction of pine oil that is rich in fenchyl alcohol. Sodium or potassium bichromate, or chromic acid, is preferable in some respects to nitric acid, since the latter converts much 80 of the pine oil into undesired products. I have employed other oxidizing agents such as chlorine, potassium permanganate and sodium hypochlorite, as well.

According to one method of oxidizing pine 85 oil, as described in my said application, the pine oil is treated with 4.2 times its weight of an oxidizing mixture consisting of 15% sodium bichromate, 20% of sulfuric acid of 60° Bé. and 65% of water, but different proportions of the oxidizing agent, as well as varying amounts of acid and water, may be employed. Agitation is employed at a temperature of 21-32° C., with some cooling, since the reaction is exothermic, but the temperature may be allowed to rise somewhat higher. The crude oxidized oil is then refined by a steam distillation.

The invention forming the subject of the present application has for its object to 100

produce oxidized pine oil products having a relatively low boiling range. It comprises in part matter divided out of said earlier application and in part is an improvement or modification of the subject-matter of said earlier application.

In said earlier application it is stated that treating oxidized pine oil with a suitable dehydrator results in the conversion of 10 a large part (say 60 per cent) of the oxidized pine oil into a lower boiling product, which, if desired, may be distilled off, leaving a residue comprising about 35 per cent of the original pine oil. As a typical example, it is stated that pine oil, oxidized as described, is heated for one and one-half hours to 150° C. with two per cent of fuller's earth. The fuller's earth is then separated from the liquid, and the latter is distilled 15 and collected in one lot. The product may be designated type A. It may be used in lacquers in much the same manner as any other oxidized pine oil, being blended with nonsolvent diluents and permissibly with 20 other nitrocellulose solvents.

The advantages of type A over simple oxidized pine oil are:

- (1) Greater volatility.
- (2) Better solvent action on nitrocellulose 30 in certain solvent mixtures.
- (3) Greater freedom from blushing in lacquers.

It is, however, a poorer solvent for certain resins than straight oxidized pine oil.

35 The following is a comparison of the boiling ranges of typical samples of oxidized pine oil and type A—

| 40           | Oxidized pine oil | Type A |     |
|--------------|-------------------|--------|-----|
|              |                   | °C.    | °C. |
| 5% over st.  | 186               | 176    |     |
| 20% over at. | 198               | 180    |     |
| 50% over at. | 208               | 186    |     |
| 70% over at. | 210               | 190    |     |
| 90% over at. | 215               | 210    |     |

45 They differ chemically chiefly in the fact that part or all of the alpha-terpineol (b. p. 218° C.) in oxidized pine oil is converted into lower boiling substances (b. p. 170-185° C.) when type A is prepared.

These lower boiling substances consist largely of terpene hydrocarbons, dipentene and others. The alpha-terpineol which is present in oxidized pine oil has little colloiding action on nitrocellulose. The active colloiding ingredients in oxidized pine oil (camphor, fenchone, etc.) are not injured if the dehydration treatment is properly applied.

50 60 An alternative way of preparing type A comprises the following steps:

- (a) The pine oil is treated with a dehydrating agent, thereby converting all or part of its terpineol content into lower boiling

point substances, but with a minimum 65 amount of dehydration of the remaining constituents.

(b) Forty to seventy-five per cent of the product is removed by distillation, preferably by using a fractionating column. 70

(c) The residual pine oil is oxidized in the manner set forth in my earlier application and as hereinbefore described or in any other efficient way.

(d) The oxidized residual pine oil is then 75 refined by steam distillation.

(e) The refined oxidized residual pine oil may be then added to part or all of the distillate from step (b), thereby obtaining the product hereinbefore designated as type 80 A having a boiling range approximating that hereinbefore specified for type A.

However, the oxidized residual pine oil resulting from step (c) may be employed 85 alone.

One particular way of practicing the modified process just described is as follows: The pine oil is heated to 145° C. for one hour with one and one-half per cent of fuller's earth. After separating the fuller's earth, 90 sixty per cent of the charge is distilled off through a fractionating column. The residue is then oxidized as hereinbefore described. The crude product is refined by steam distillation and is then blended with 95 the first distillate.

It should be stated that in referring to a dehydrator or dehydrating agent, I intend to include any reagent, some of which are hereinafter mentioned, whose chief effect is that of splitting off chemically combined water from certain of the pine oil constituents, notably terpineol. A wide variety of dehydrators may be employed, in either described method, but it is preferable to use one which decomposes the terpineol without attacking the other constituents. If the second described method is employed, somewhat more care is necessary in carrying out the dehydration. Mineral acids, e. g. dilute sulfuric acid, acid salts (e. g. sodium bisulfate), salts which give an acid reaction on hydrolysis (e. g. copper sulfate), small amounts of iodin or bromin, or various substances which dehydrate by virtue of surface catalysis, may be employed. The latter class includes activated carbon, fuller's earth, kieselguhr, and in some instances other argillaceous or silicous earths. 115

While, in the foregoing description, I 120 have described the process as starting with pine oil as the raw material, it should be understood that I mean to include, as an equivalent for pine oil, the by-product oil which is obtained in preparing terpin hydrate from pine oil.

The foregoing discussion of methods of dehydration applies to dehydration in the

liquid phase. Dehydration of the pine oil, before or after oxidation, may also be carried out in the vapor phase by passing the vapors over heated aluminum oxide, phosphoric acid on coke, or any of the catalysts which are employed in the dehydration of alcohols.

Type A, like straight oxidized pine oil, will contain a proportion of oxidized inert bodies, serving as diluents, and in preparing the nitrocellulose solution, it is usually desirable, as when using straight oxidized pine oil, to add rather large proportions of lower boiling liquids, which may be solvents or non-solvents for nitrocellulose.

The special oxidized pine oil products hereinbefore described as embodying the present invention have, except for their lesser capacity to dissolve certain resins, all the advantages of oxidized pine oil products produced by simple oxidation of their oxidizable constituents, and in addition have the advantages, hereinbefore mentioned, of greater volatility, better solvent action on nitrocellulose in certain solvent mixtures, and greater freedom from blushing in lacquers; and are therefore preferred by many users.

Where reference is made to a nitrocellulose lacquer, I do not mean to include only those lacquers which contain resins, as the oxidized product is also applicable as a nitrocellulose solvent when resins are not present in the solution, and in fact, in the latter case, the product embodying my invention is of special advantage.

When, in the claims covering my new process, I specify certain steps, particularly oxidation and dehydration, I do not mean to be confined to practicing the steps in the order recited, except in those claims where the language is obviously intended to be limited to the order in which the steps are practiced.

Having now fully described my invention, what I claim and desire to protect by Letters Patent is:

1. A pine oil product adapted for use in preparing a solvent for nitrocellulose, comprising dehydrated constituents and oxidized constituents of pine oil adapted to have a substantial colloiding action on nitrocellulose.

2. A pine oil product adapted for use in preparing a solvent for nitrocellulose, comprising dehydrated constituents and oxidized constituents of pine oil adapted to have a substantial colloiding action on nitrocellulose, and inert constituents of pine oil acting as a diluent.

3. A pine oil product adapted for use in preparing a solvent for nitrocellulose, comprising dehydrated constituents and oxidized constituents of pine oil adapted to have a substantial colloiding action on nitrocellulose, and a diluent having a substan-

tially lower boiling range than the boiling range of oxidized pine oil.

4. A pine oil product adapted for use in preparing a solvent for nitrocellulose, comprising dehydrated constituents and oxidized constituents of pine oil adapted to have a substantial colloiding action on nitrocellulose, a diluent liquid having a substantially lower boiling range than the boiling range of oxidized pine oil, and inert constituents of pine oil also acting as a diluent.

5. A pine oil product adapted for use in preparing a solvent for nitrocellulose comprising dehydrated constituents and oxidized pine oil adapted to have a substantial colloiding action on nitrocellulose and the preponderating proportion of whose constituents has a boiling range of approximately 175-220° C.

6. The process of preparing pine oil for use in the preparation of a nitrocellulose lacquer which comprises subjecting pine oil to two treatments: Namely, treatment with a dehydrating agent to convert certain constituents into a lower boiling product, and treating with an agent effective to oxidize certain oxidizable constituents of the pine oil.

7. The process of preparing pine oil for use in the preparation of a nitrocellulose solvent, which comprises subjecting pine oil to two treatments: Namely, treatment with a dehydrating agent to convert certain constituents into a lower boiling product followed by distillation, and treating with an agent effective to oxidize certain oxidizable constituents of the pine oil followed by distillation.

8. The process of preparing pine oil for use in the preparation of a nitrocellulose solvent, which comprises first treating pine oil with a dehydrating agent to convert certain constituents thereof into a lower boiling product, and then treating the dehydrated product with an agent effective to oxidize certain oxidizable constituents thereof.

9. The process of preparing pine oil for use in the preparation of a nitrocellulose solvent, which comprises first treating pine oil with a dehydrating agent to convert certain constituents thereof into a lower boiling product, then distilling off a substantial percentage of the dehydrated product, then treating the residual product with an agent effective to oxidize certain oxidizable constituents thereof, and then refining the oxidized product by distillation.

10. The process of preparing pine oil for use in the preparation of a nitrocellulose solvent, which comprises first treating pine oil with a dehydrating agent to convert certain constituents thereof into a lower boiling product, then distilling off a substantial percentage of the dehydrated product, then treating the residual product with an agent

effective to oxidize certain oxidizable constituents thereof, and then blending the oxidized product with said distillate.

11. The process of preparing pine oil for use in the preparation of a nitrocellulose solvent, which comprises first treating pine oil with a dehydrating agent to convert certain constituents thereof into a lower boiling product, then distilling off a substantial percentage of the dehydrated product, then

treating the residual product with an agent effective to oxidize certain oxidizable constituents thereof, then refining the oxidized product by distillation, and then blending the refined residue with distillate produced in the second of the foregoing steps.

In testimony of which invention, I have hereunto set my hand at Kenvil, New Jersey, on this 12th day of Aug., 1925.

IRVIN W. HUMPHREY.